

Patented May 6, 1930

1,757,805

6

Soy bean + aqueous solution + KM

## UNITED STATES PATENT OFFICE

IRVING F. LAUCKS AND CHARLES N. CONE, OF SEATTLE, WASHINGTON, ASSIGNEES  
TO I. F. LAUCKS, INC., OF SEATTLE, WASHINGTON, A CORPORATION OF WASHING-  
TON

## PROCESS OF MANUFACTURE OF GLUE AND THE PRODUCT THEREOF

No Drawing.

Application filed September 13, 1924. Serial No. 737,576.

Our invention relates to the manufacture of adhesive materials, and more particularly materials adaptable to large scale application, for instance as adhesives in making up 5 ply wood, veneers, and the like.

In providing a glue for use in the manufacture of ply wood for instance, certain limiting conditions must be met. Obviously, a primary characteristic of a suitable glue for 10 such use is the strength of bond which it provides. Another necessary quality is workability in mixing and spreading machines, etc., and furthermore the glue after mixing should retain its adhesive properties for a 15 sufficient time to allow of delays which may be incurred before application. Moreover it is often desired to change the proportion of the ingredients of a particular batch of glue for which the dry mixture is already prepared, in order to meet the requirements of 20 a different wood or the like to be glued. It is desirable also that the material be available at a minimum cost.

To the accomplishment of the foregoing 25 and related ends, the invention, then, consists of the features hereinafter fully described, and particularly set forth in the claims, the following description reciting certain illustrative forms of the invention, which obviously are but a few of the various ways in 30 which the principle of the invention may be employed.

In carrying out our invention, a preferable procedure is as follows: A dry, finely ground 35 vegetable protein-containing-material, such as oil seed cake and preferably ground soya bean cake or if desired, the powdered material obtained by extracting the protein from soya beans or soya bean cake, is mixed with hydrated lime, powdered rosin, or other resin or compounds of resins with sodium, calcium 40 or other metals; a manganese compound such as manganese dioxide, manganese sulphate, or potassium permanganate or their equivalents 45 capable of furnishing available manganese is added; to these dry mixed ingredients there is then added in a suitable mixing apparatus a proper amount of water, either hot or cold, that is, as customarily understood, 50 hot water for instance being not to exceed

about 120° F. and cold water from about 60° F. down to freezing. When the ingredients are well mixed, a suitable amount of caustic soda, as ordinarily the most available and cheapest alkali, is added in aqueous solution 55 and the mixing continued; then a suitable quantity of sodium silicate solution is added having regard to the consistency requirements of the material upon which the adhesive is to be used, whether wood or paper 60 or other material, and whether moist or dry, etc. After the mixture has reached a proper consistency, as evidenced to those experienced in the art by its color, stringiness, etc.,—the signs by which those experienced in the art 65 of vegetable protein glue use are enabled to judge of its consistency,—the glue is ready for application to ply wood and veneer, etc. in the customary manner.

If desired, the water soluble compounds of 70 manganese may be omitted from the dry mix and be added directly in the initial water, which may be hot or cold as desired, or the manganese compounds may be added in water solution after the addition of sodium sili- 75 cate to the mix.

As examples, the following illustrative formulae are cited:

(1) Mix 180 parts ground soya bean cake with 30 parts hydrated lime, and, 30 parts 80 ground rosin and from  $\frac{1}{2}$  part to 10 parts of potassium permanganate; add to 600 to 700 parts water, and mix well; add 5 to 30 parts of a 40% caustic soda solution and stir well; add 90 parts sodium silicate solution about 40° Baumé and stir well; add sufficient water, 300 to 400 parts, to bring to proper consistency, giving finished glue.

(2) Proceed as in No. 1 above, except that in place of potassium permanganate use from 90 10 to 30 parts of manganese dioxide.

(3) Proceed as in No. 1 above, except that in place of potassium permanganate use from 95 5 to 20 parts of manganese sulphate.

Rosin and sodium silicate being agents in the nature of spreaders are of course not desired in every case; depending, as indicated, on the conditions under which the adhesive is to be used.

Other modes of applying the principle of 100

our invention may be employed instead of the one explained, change being made as regards the details herein disclosed, provided the procedure or the ingredients stated by 5 any of the following claims or the equivalents of such stated procedure or ingredients be employed.

We therefore particularly point out and distinctly claim as our invention:—

- 10 1. An adhesive material embodying vegetable protein containing material derived from oleaginous seeds, in aqueous alkaline media, and a manganese compound.
- 15 2. An adhesive material embodying vegetable protein containing material derived from oleaginous seeds, in aqueous alkaline media, and a manganese compound in the proportion range of approximately 11/100 per cent to approximately 17 per cent of such 20 compound, such percentage being based on the weight of such vegetable protein containing material.
- 25 3. An adhesive material embodying vegetable protein containing material derived from soya beans, in aqueous alkaline media, and potassium permanganate.
- 30 4. An adhesive material embodying vegetable protein containing material derived from soya beans, in aqueous alkaline media, and potassium permanganate in the proportion range of approximately 11/100 per cent to approximately 5.5 per cent, such percentage being based on the weight of such vegetable protein containing material.
- 35 5. An adhesive material embodying vegetable protein containing material derived from soya beans, and lime, and caustic soda and water, and potassium permanganate.
- 40 6. An adhesive material embodying vegetable protein containing material derived from soya beans, and lime, and caustic soda and rosin, and water, and potassium permanganate.
- 45 7. An adhesive material embodying vegetable protein containing material derived from soya beans, and caustic soda and water and sodium silicate and potassium permanganate.

In witness whereof, we hereunto subscribe 50 our names this 3d day of Sept., 1924.

IRVING F. LAUCKS.  
CHARLES N. CONE.